

# UNITED STATES PATENT OFFICE.

LEO H. BAEKELAND, OF YONKERS, NEW YORK, ASSIGNOR TO DEVELOPMENT AND FUNDING COMPANY, OF NEW YORK, N. Y., A CORPORATION OF NEW JERSEY.

## ELECTROLYTIC DIAPHRAGM AND METHOD OF MAKING SAME.

No. 855,221.

Specification of Letters Patent.

Patented May 28, 1907.

Application filed March 10, 1906. Renewed February 16, 1907. Serial No. 357,756.

*To all whom it may concern:*

Be it known that I, LEO H. BAEKELAND, a citizen of the United States, residing at Yonkers, in the county of Westchester and State of New York, have invented certain new and useful Improvements in Electrolytic Diaphragms and Method of Making Same, of which the following is a specification.

The object of this invention is to provide a diaphragm for electrolytic purposes and specifically for use in the electrolysis of brine.

The diaphragm may be made of any desired porosity, and its porosity may be afterward modified if occasion therefor should arise: it contains no materials which are subject to solution or attack by brine or by the electrolytic products thereof, and is furthermore strong, flexible and durable. In these respects it is superior to any diaphragm of which I am aware.

My improved diaphragm is more particularly intended for use in the electrolysis of brine under such conditions that a limited quantity of brine is permitted to percolate from the anode compartment to the region of the cathode where the production and separation of caustic soda occurs, as, for instance, in an electrolytic cell of the type described in U. S. Patent 779,383, issued January 3, 1905, to Clinton Paul Townsend. In a cell of this character it is desirable that the diaphragm should possess a substantially uniform porosity in order that the concentration of the caustic may be substantially uniform over the entire area of the cathode. It is furthermore desirable that the diaphragm should be capable of production in large sheets or surfaces, and that it should be of sufficient strength to permit it to be cleaned mechanically without injury. All of these requirements are fulfilled by a diaphragm made in accordance with my invention.

A preferred form of diaphragm is made as follows: To the surface of a base consisting of woven asbestos fabric, commonly known as asbestos cloth, I apply a permeable coating, paste or paint, consisting of an oxid of iron such as Venetian red or Indian red, asbestos powder or equivalent filling material, and a cementing material or binder which preferably consists of ferric or ferrous hydroxid. This paint may be prepared by pre-

cipitating 400 cc. of ferric chlorid solution having a specific gravity of about 1.4 by an excess of caustic soda, and adding to the resulting alkaline mass and thoroughly incorporating therewith about 500 grains of ferric oxid and 1,200 grains of asbestos powder, together with sufficient water to convert the mixture into a rather thick paint. Such mixture is uniformly spread over the asbestos cloth and permitted to dry thereon, when the diaphragm is ready for use.

The excess of caustic soda above referred to is desirable as it distinctly aids by its cementing effect in the production of a coherent and durable coating.

I regard ferrous hydroxid as the equivalent of ferric hydroxid for my purpose inasmuch as it becomes wholly or partly converted into ferric hydroxid during the drying of the diaphragm. It possesses over ferric hydroxid the advantage of economy since it is readily prepared by dissolving scrap iron in commercial muriatic acid and precipitating the resulting ferrous chlorid solution.

I do not limit myself to the specific ingredients or proportions above noted as preferred. The asbestos cloth is in itself quite pervious and its interstices are quite irregular in size and distribution, rendering it entirely unsuited for my purpose. In the formation of my diaphragm it is necessary that these interstices be filled or covered by an adherent and permeable coating which is substantially unaffected under the conditions of use. The use of organic materials should be avoided.

My diaphragm differs entirely from sized asbestos sheets or paper heretofore used for such purposes. Such sheets are difficult to handle without injury even when dry, and when wet are reduced to a pulp having no coherence; it is impossible to clean them by mechanical means. The size employed being organic and usually of a starchy character swells when wet, therefore reducing the permeability of the diaphragm; such size is furthermore subject to attack by the solution and the products of electrolysis.

I claim:

1. A diaphragm comprising a pervious base and a permeable coating or filling dried thereon, substantially as described.

2. A diaphragm comprising a base of woven fabric and a permeable coating or filling dried thereon, substantially as described.
3. A diaphragm comprising a base of asbestos cloth and a permeable coating or filling dried thereon, substantially as described.
4. A diaphragm comprising a pervious base and a permeable coating or filling dried thereon, said coating containing an oxid of iron and a binder, substantially as described.
5. A diaphragm comprising a base of asbestos cloth and a permeable coating or filling dried thereon, said coating containing an oxid of iron and a binder, substantially as described.
6. A diaphragm comprising a base of asbestos cloth and a permeable coating or filling applied thereto, said coating containing an oxid of iron, a filling material and a binder substantially as described.
7. A diaphragm comprising a base of asbestos cloth, and a permeable coating or filling applied thereto, said coating containing an oxid of iron, asbestos and a hydroxid of iron, substantially as described.
8. A diaphragm comprising a base of asbestos cloth and a permeable coating or filling applied thereto, said coating comprising an alkaline mixture of ferric oxid, asbestos, and a hydroxid of iron, substantially as described.
9. The method of making a diaphragm which consists in applying to a pervious base a permeable coating or filling, and drying it thereon, substantially as described.

In testimony whereof, I affix my signature in presence of two witnesses.

LEO H. BAEKELAND.

Witnesses:

THOMAS W. IVERS,  
JOHN J. STAHL.